

March 4, 1941.

E. LUKÁCS

2,233,869

COLD WORKING METAL BAR

Filed Jan. 13, 1939

2 Sheets-Sheet 1.



INVENTOR

ERNST LUKÁCS

BY *Richards & Geier*

ATTORNEYS

March 4, 1941.

E. LUKACS

2,233,869

COLD WORKING METAL BAR

Filed Jan. 13, 1939

2 Sheets-Sheet 2



Fig. 7.



Fig. 8.



Fig. 9.

INVENTOR  
ERNST LUKACS  
BY *Richard S. Geier*  
ATTORNEYS

## UNITED STATES PATENT OFFICE

2,233,869

## COLD WORKING METAL BAR

Ernst Lukács, Budapest, Hungary

Application January 13, 1939, Serial No. 250,737  
In Hungary October 9, 1937

## 6 Claims. (Cl. 29—1)

My invention relates to metal bars and more particularly to a method of an apparatus for cold working round, or nearly round, metal bars of commercial quality, such as round iron rods, by means of twisting.

The expression "round or nearly round metal bars" used hereinafter, does not include bars provided with projections such as ribs, for example section or profiled iron, and the invention 10 is not to be construed as including the treatment of such bars.

In the case of most metals, when they are worked in the cold state, without removing particles of matter, in such a way that the individual 15 particles of matter are mutually displaced, it is known that the yield point and tensile strength are raised, while stretching is lowered. Such working is of particular importance in the case of the ordinary round iron rods of commerce 20 which are embedded in a foreign medium, such as concrete, and subjected to tension.

The degree of working, and hence the raising of the yield point and so on, could not hitherto be ascertained from iron rods so worked. It was 25 therefore necessary to proceed very carefully when using iron rods treated in this manner, so that the stressing to which they were subjected generally remained far below the permissible limit.

30 The object of my invention is to provide cold worked iron rods with markings indicative of the degree of improvement bestowed by cold working.

A further object of my invention is to produce 35 such markings simultaneously with the cold working operation. Still another object of my invention is to utilize the tools by which the rods are cold worked for producing simultaneously said markings.

My invention comprises a method of and an 40 apparatus for marking metal bars and may be used when round, or nearly round, metal bars are subjected to twisting in the cold state, for example are gripped at one end and turned at the other until they undergo permanent deforma- 45 tion.

I provide the round or nearly round metal bar, such as a round iron rod, to be worked by means 50 of twisting, either before or at the same time as it is so worked, with a marking which represents, after the working, a pattern in the shape of a helical line, the pitch of which is substantially inversely proportional to the degree of working, while this proportion may be either linear or non-linear.

55 My invention may, for example, be carried out

by providing on the metal bar, before it is worked, small impressions, such as fluting or milling, running parallel to the axis of said bar, which assume the form of a helical line when the bar undergoes twisting. The impressions may naturally be replaced by any other desired markings, for example coloring or the like. The pattern which appears after the working may be of any type, while any two points can be fixed on the pattern between which the pitch of the helical 10 line is measured.

The advantage of my method consists in that 15 patterns are produced on the outer surface of the metal bar which enable the yield point and tensile strength of the bar to be deduced with certainty. My method also affords the additional advantage that the regularly distributed uneven portions of the surface of the bar substantially increase the adhesion of the iron rod in the embedding medium, such as concrete.

20 Various apparatus can be employed for carrying out the method of the invention, i. e. for twisting the iron rod and marking the degree of torsion, and of these the following will be described by way of example:

The metal bar is drawn through a pair of loaded rolls, one or both of which are grooved, or through a grooved tool, and then one end of the bar is gripped in a stationary jaw while the other end is turned until the desired increase in 30 the yield point has taken place. The degree of torsion can be measured with a revolution counter, which in turn can be coupled, if desired, with a per se known automatic disconnecting device, by which the apparatus used for twisting the bar is automatically disconnected when the desired screw pitch is attained.

The metal bar is passed between rolls, one or 35 both of which are grooved and the axes of which are not parallel, being drawn therethrough either on a draw bench, by means of gripping pliers, or with the aid of a pair of rolls. The gripping pliers should not perform any rotary movement.

The metal bar is drawn through a pair of driven 40 rolls one or both of which are grooved and which also perform a planetary movement about the axis of the bar, while in this case also the bar can be drawn therethrough with the aid of gripping pliers or of a pair of rolls.

45 In order that the invention may be more clearly understood, reference is made to the accompanying drawings, in which:

Fig. 1 is a diagrammatic side elevation of one embodiment of my apparatus;

Fig. 2 is a sectional view of the same along the line II—II of Fig. 1;

Fig. 3 is a view of a marked metal bar before the twisting operation;

5 Fig. 4 shows the same bar after the twisting operation;

Fig. 5 is a side elevation of a second embodiment of my apparatus;

Fig. 6 is a top view of the same;

10 Fig. 7 is a side elevation, partly in section, of a third embodiment of my apparatus;

Fig. 8 is a top view of the same;

15 Fig. 9 is a characteristic curve showing the improvement of the mechanical properties as a function of the degree of twist.

In Figs. 1 and 2 is shown the simplest form of the apparatus, in which a pair of rotary rolls, consisting of a grooved upper roll 1 and an even lower roll 2, is employed, the upper roll 1 being mounted with its axis 17 in a pair of levers 18 pivoted at 19 on a bracket 20 constituting a part of the supporting frame 21. The levers 18 support a weight 3, so that the upper roll 1 is constantly pressed against the lower roll 2. The 20 axis 22 of the lower roll 2 is rotatably mounted in stationary bearings 23 which form a part of the frame 21. If a round iron rod *g* be now drawn through the pair of said rolls in any desired direction, the groovings provided on the upper 25 roll will be impressed into the iron rod, as shown in Fig. 3. In the marking apparatus shown in Figs. 1 and 2, a pair of rolls 24, 25 are used to move the rod *g* forward between the marking rolls 1 and 2. The forwarding rolls 24, 25 are 30 rotatably mounted in alignment with the marking rolls 1 and 2, the lower roll 25 having stationary bearings, while the upper roll 24 is journaled in a bearing block 42 which is slidably mounted in the frame 21 and is engaged by a coiled spring 26, the tension of which may be 35 adjusted by a set screw 27. The rolls 24 and 25 are rotated with equal peripheral speeds by toothed wheels 24' and 25', respectively, which mesh with one another and with a pinion 28 driven by a motor not shown in the drawings. If 40 the rod *g* which leaves the apparatus shown in Figs. 1 and 2 with the marking *i* impressed upon it (Fig. 3), is then subjected to torsion until permanent deformation takes place, the impressed 45 depressions *i* on the surface of the iron rod will form a pattern running in the form of a helical line, as will be apparent from Fig. 4. The pitch *e* of the helical line is substantially inversely proportional to the degree of working and can be 50 limited with the aid of an automatic disconnecting device.

In the embodiment illustrated in Figs. 5 and 6, the apparatus comprises gripping pliers 5 and grooved rotary rolls 6, 7, the axes 8, 9 of which 55 are not parallel to one another but lie in parallel planes. The axes 8 and 9 of the rolls 6 and 7 are journaled in bearing blocks 29 and 30, respectively, said blocks being slidably mounted in the supporting frame 31 and carried by 60 adjustment screws 32 extending through openings formed in the frame 31 and having inner screw threads. The screws 32 are rotatably connected with the bearing blocks 29 and 30. By 65 turning the adjustment screws 32, the rolls 6 and 7 may be pressed against the rod *g*. Gripping pliers 5 are then used to move the rod forward between the rolls. In order to prevent 70 the rod from rotating, the pliers 5 are connected by a pair of links 33 and a bifurcated link 34 to a block 35 which is guided along with two

75 pairs of lateral rollers 36 between two stationary guide rails 37, which are U-shaped in cross-section. The block 35 is drawn by a chain 38 in the direction of the arrow 10, so that it moves in the longitudinal direction of the rod *g*. When the 80 rod is thus drawn between the rolls 6 and 7 and is wedged between them with suitable pressure, it will be subjected to a torsion which is proportional to the inclination of the roll axes to one another. The grooving on the rolls 6, 7 85 is impressed into the iron rod, so that patterns running in the form of a helical line will be produced on the iron rod. The pitch of the helical line is once again substantially inversely proportional to the deformation of the iron rod, 90 i. e. to the degree of torsion.

Finally, the apparatus in the example shown in Figs. 7 and 8 consists of gripping pliers 11 and a grooved upper roll 12 and an even lower roll 13, the axes 14, 15 of which are parallel and 95 which, in addition to their rotation about their own axes, also revolve about the axis of the iron rod *g*. For this purpose the rolls are mounted in a trunnioned frame 16 rotatably mounted in a pedestal 17. The trunnions 39 of the frame 16 100 are hollow, so that the rod *g* can be moved through them to and from the rolls 12 and 13. The frame 16 is rotated by a toothed wheel 40 which is fixed upon one of the trunnions 39 and meshes with a pinion 41. The pinion 41 105 is journaled in the pedestal 17 and is driven by a motor not shown in the drawings. The gripping pliers 11 as well as other elements drawing the rod between the rolls 12 and 13 are identical to those provided in the device illustrated 110 in Figs. 5 and 6 of the drawings. If the iron rod *g* be now drawn by means of the gripping pliers 11 (or by means of a pair of rolls) between the rolls 12, 13, in the direction of the arrow 18, it will undergo torsion in a similar way as in 115 the example shown in Figs. 4 and 5, and at the same time patterns in the form of a helical line will be produced on its surface and will be indicative of the degree of torsion.

The raising of the yield point or of the tensile 120 strength can be represented, as shown in Fig. 9, in the function of a fraction *e/D*, the numerator *e* of which represents the pitch of the helical line appearing after the working and the denominator *D* of which represents the diameter of 125 the metal bar. From the inspection of the curve *F* in Fig. 9 it will be seen that the yield point rises as the fraction *e/D*, i. e., with bars of the same diameter *D* the pitch *e* of the helical line 130 decreases.

The method of the invention is also suitable 135 for marking round or nearly round metal bars the tensile strength of which varies in the direction of the length by twisting the bar according to a helical line of varying pitch, for example 140 with the aid of the apparatus illustrated in Figs. 5 to 8, the pattern appearing on the surface of the bar after the working automatically and immediately indicating the varying tensile strength. On the contrary, variation of the pitch of the 145 helical line along a bar which has been twisted in a uniform manner throughout its length indicates that the bar was originally defective, i. e. of varying resistance against torsional stress.

15 I claim:

1. In a method of cold working roundish metal bars by twisting, the step of furnishing the surface of the bar with a marking so running in longitudinal direction as to extend on the twisted bar along a helical line, the pitch of which is 155

characteristic of the degree of working bestowed by twisting.

2. In a method of cold working roundish metal bars by twisting, the step of furnishing the surface of the bar with impressions so running, in longitudinal direction as to extend on the twisted bar along a helical line, the pitch of which is characteristic of the degree of working bestowed by twisting.

10 3. In a method of cold working roundish metal bars by twisting, the step of furnishing the surface of the bar before the twisting operation with a marking running parallel to the axis of the bar so as to extend on the twisted bar along a helical line, the pitch of which is characteristic of the degree of working bestowed by twisting.

15 4. In a method of cold working roundish metal bars by twisting, the step of furnishing the surface of the bar before the twisting operation with 20 impressions running parallel to the axis of the

bar so as to extend on the twisted bar along a helical line, the pitch of which is characteristic of the degree of working bestowed by twisting.

5 5. In a method of cold working roundish metal bars by twisting, the step of furnishing the surface of the bar simultaneously with the twisting operation with a marking so running in longitudinal direction as to extend on the twisted bar along a helical line, the pitch of which is characteristic of the degree of working bestowed by 10 twisting.

15 6. In a method of cold working roundish metal bars by twisting, the step of furnishing the surface of the bar simultaneously with the twisting operation with impressions so running in longitudinal direction as to extend on the twisted bar along a helical line, the pitch of which is characteristic of the degree of working bestowed by 15 twisting.

ERNST LUKÁCS. 20